

## UNITED STATES PATENT OFFICE

2,040,430

## ART OF STABILIZING SOAP

Ernest C. Crocker, Belmont, and Lloyd F. Henderson, Reading, Mass., assignors to Arthur D. Little, Incorporated, Cambridge, Mass., a corporation of Massachusetts

No Drawing. Application December 11, 1928,  
Serial No. 325,381

7 Claims. (Cl. 87—16)

This invention relates to a process of stabilizing soap in respect both to color and odor. The tendency of soap, especially white soap, to take on with age a yellowish color, either uniformly throughout or in yellowish or brownish spots or streaks, to lose its perfume and otherwise change its odor, is well known, and it is the object of the present invention to obviate these objectionable results. Such discoloration and change of odor have been generally attributed to oxidation of some of the ingredients of soap by the oxygen of the air, but the cause and mechanism of the oxidation and the nature of the resulting deleterious effects have been obscure.

We have discovered that this oxidation is promoted principally by the catalytic action of certain multivalent metals. Soap always contains traces of multivalent metals, especially copper and iron, which are harmful, and often zinc, nickel, lead and tin, which are relatively non-injurious. Such metals come from various sources. They may be picked up from the apparatus used in making the soap, or from the vats and containers for the ingredients from which the soap is made. They are present to some extent in the original ingredients as a customary or as a natural impurity; for example, caustic soda and certain vegetable oils contain copper. Many soap fats are derived from waste sources and are more or less badly contaminated with metals; and many perfume materials contain copper and sometimes other metals. But from whatever sources the metals may come, a soap stock is practically never free from traces of multivalent metals.

The principal deleterious metals are the multivalent metals, copper and iron; the others are apparently negligible from the point of view of discoloration and loss or change of odor. Copper and iron are normally present in the soap though only in minute quantities. While the amounts vary widely in different soap stocks, they are commonly found in quantities of the order of one part of copper to from one million to fifty million parts of soap, and one part of iron to several hundred thousand parts of soap. But even in minute quantities of this order they produce discoloration and change of odor. Quantities of copper too small to be detectable by ordinary analytical procedures can cause marked failure of color and odor. For example, when two parts of copper per million parts of soap are intentionally added, the effects are soon detected, and are far more severe than is usually found in

practice. It is to be understood that the foregoing proportions are merely illustrative of normal and typical conditions, and of the nature of the problem, and are by no means intended to define any uniform or standard condition nor any limitation to which the invention is confined. The presence of the metals in larger quantities than suggested as typical is, of course, even more injurious, and even in very much smaller quantities produces appreciable deleterious effects in the soap. Iron may be, and usually is, present in greater quantity than copper, but we have observed that quantity for quantity copper is a vastly more important factor than iron in promoting oxidation. Both, however, when present, are amenable to the present invention.

We have discovered that copper and iron cations promote oxidation of certain ingredients of the soap. The presence of ions implies the presence of water or equivalent ionizing material. Soap always contains water. The oxidation is characterized by the development of rancidity, which in turn is accompanied by a darkening of the soap and by an unpleasant odor. Alteration and weakening of the perfume is also a result of such oxidation. It is the aim of the present invention therefore to remove the cause of the objectionable oxidation by substantially eliminating the copper and iron ions (cations) and hence nullifying the oxidation-promoting action of the metals. It is obviously not practicable physically to remove from the soap the copper and iron which are present in such exceedingly minute quantities, but we have succeeded in removing the oxidation-promoting cation form of these metals by chemical means.

This we have accomplished in two ways: first, by precipitating the copper and iron; second, by forming complexes of the copper and iron wherein the properties characteristic of the metal cations are absent. Both methods may be termed demetalization or de-ionization, by which we mean the substantial elimination of metal cations, that is, the decrease of the concentration of metal cations to the point where they are incapable of appreciable oxidation-promoting action.

In carrying out the precipitation method, which is our preferred method, we add to the soap a reagent which forms with the copper and iron, in the presence of soap, a sufficiently insoluble precipitate so that the amount of metals remaining in solution as cations is negligible, thus eliminating the activating or promoting

cause of oxidation. This precipitate to be effective is necessarily less soluble, and hence forms fewer ions in the presence of soap, than do the soaps of the metals. Of a number of precipitating materials effective for the purpose we prefer zinc sulfide, which may be introduced either into the neat soap as it comes from the kettle, or, when a milling process is used (the so-called "French" process), is preferably introduced into the mixer preparatory to the milling. This material, while it may be considered, properly, as "insoluble", is vastly more soluble than are the sulfides of iron and copper and hence is able to precipitate traces of iron and copper from soap, as the sulfides, particularly when it is present in excess of the amount needed for such precipitation.

By way of specific example of the application of the invention to the milling process of making soap the following procedure is recommended. Neat soap as it comes from the kettle in hot, viscous-liquid form containing approximately 70% soap and 30% water, is chilled on rolls, from which it comes in the form of moist shavings or sheets; the moist shavings are then placed in a drier and dried; from the drier the dried shavings are passed into a mixer in which they are worked into a dough-like consistency by a kind of churning action. The perfume materials are usually introduced into the mixer, and it is preferably at this stage also that we introduce the precipitating agent. Zinc sulfide, the preferred precipitating agent, in the form of a white powder and in the proportion of about .4% of the soap by weight, is put into the mixer and there thoroughly mixed with and dispersed throughout the soap mass. The quantity of precipitant thus recommended is in excess of that theoretically necessary to precipitate the small amounts of soluble copper and iron normally present, but such excess is desirable as it furnishes a reserve of precipitating material against any emergency, such as the presence of more copper or iron than was expected, or later contamination by further processing, from wrappers, etc., or the effects of atmospheric oxidation on the sulfide precipitates formed, in case the iron precipitate, for example, should slowly oxidize to sulfate by the action of atmospheric oxygen. In any of these events the excess of zinc sulfide, or other precipitating agent used, will react with the stabilized metal and again precipitate it.

After the soap leaves the mixer it is passed through the several mills, the plodder, the cutter and the press according to usual practice.

Other reagents beside zinc sulfide which, when added to copper and iron in alkaline solution, will form precipitates and act as eliminators of the copper and iron ions, are sodium and other water soluble sulfides, such sulfur derivatives as can form sulfides in the presence of copper and iron in soap, and other precipitants for traces of iron and copper in the presence of soap. Examples are lithopone, cryptone, methylene blue and thiourea.

In general, any material which forms compounds of copper and iron which are less soluble in soap than are copper and iron soaps will act more or less well as a precipitant for this purpose. Methylene blue and thiourea are instances of organic compounds, which in time decompose, giving off hydrogen sulfide, which is the actual precipitant.

As already mentioned, instead of adding the precipitating agent to the soap in the mixer, it

may be added to the neat soap as made in the kettle. While this is an alternative (and less desirable) procedure in the manufacture of soap by the milling process, it is the only practicable procedure in the manufacture of soap by the ordinary "frame" process since in the frame process all steps from the chilling rolls to the plodder, both inclusive, are omitted and replaced by solidifying the neat soap in the frame and dividing it into bars preparatory for the cutting of it into cakes. Therefore the only feasible stage of the frame process for introducing the precipitating agent is into the fluid or semifluid neat soap before it goes to the frame.

The other method of demetalization, or decreasing the concentration of metal ions sufficiently to nullify their oxidation-promoting action, is by forming complexes which either do not ionize at all, or if they ionize, do so with the metal in the complex ion, which is preferably the anion. Suitable reagents for such complex formation are: sodium salicylate and the organic salicylates; eugenol and a number of other phenols; water-soluble cyanides, and arsenites; alkali salts of lactic, citric and tartaric acids; dimethyl glyoxime; thiourea; most sugars, but not sucrose; and sodium sulfosalicylate.

Any of these reagents when introduced into the soap, either in the mixer if the milling process is used, or into the neat soap from the kettle whether in the milling process or the frame process, will result in the conversion of the traces of copper and iron ions in the soap into complexes wherein the metals are inactive and the oxidation-promoting properties characteristic of the simple metal cations are absent.

Sodium salicylate has been found to combine with copper and iron compounds, at the alkalinity of soap, to make metal complexes which exist as highly colored solutions. These give none of the ordinary ionic reactions of the metals such as rapid precipitation by ferrocyanides or even by sulfides. The amounts of metals ordinarily present in the soap, however, are not enough to color the cakes of soap appreciably.

The elimination of the ions of copper and iron as above described, whether by precipitation to remove the metal ions from solution in insoluble form, or by complex formation when a soluble, un-ionized metal compound without the ordinary metal cations is formed, eliminates the cause of the catalytic oxidation-promoting action and consequently the oxidation of the ingredients of the soap and thereby prevents the development of rancidity with its resulting discoloration, change of odor and loss of perfume.

The process of demetalization herein described, which operates by eliminating the cause of oxidation by eliminating the ions of certain multivalent metals responsible for the catalytic promotion of oxidation, is to be sharply distinguished from the use of the so-called anti-oxidants, which have been proposed, at least experimentally, to lessen the ordinary oxidation which occurs in soap without removing its cause.

Our process of stabilizing, protecting and preserving soap may easily and economically be applied to existing methods of making fine toilet soaps, and is applicable as well to the manufacture of common laundry and washing soaps.

It is our purpose herein to claim the invention generically, and also to claim that species characterized by precipitation. The alternative species characterized by complex formation is not

herein claimed except as it exemplifies the genus.

We claim:

5 1. The art of stabilizing soap containing an ionized metal which acts catalytically to promote oxidation of ingredients of the soap, which comprises adding to the soap mass zinc sulfide.

10 2. That step in the milling process of making soap, which consists in adding a sulfide to the plastic soap during the mixing operation preceding the milling operation.

3. That step in the milling process of making soap, which consists in adding zinc sulfide to the plastic soap during the mixing operation preceding the milling operation.

4. The art of stabilizing soap containing ionized copper and iron, which comprises adding an excess of sulfide to the soap mass.

5 5. The art of stabilizing soap containing ionized copper and iron, which comprises adding an excess of zinc sulfide to the soap mass.

6. The art of stabilizing soap containing ionized copper, which comprises adding to the soap mass an excess of sulfide.

10 7. The art of stabilizing soap containing ionized copper, which comprises adding an excess of zinc sulfide to the soap mass.

ERNEST C. CROCKER.  
LLOYD F. HENDERSON.